

## [54] LUBRICANT FOR A CONTROLLED-SLIP DIFFERENTIAL

[75] Inventors: David S. Gates, Swarthmore; Paul E. Hagstrom, Valley Forge; Marcus W. Haseltine, Jr., Brookhaven, all of Pa.

[73] Assignee: Sun Research and Development Co., Philadelphia, Pa.

[22] Filed: Jan. 17, 1972

[21] Appl. No.: 218,394

[52] U.S. Cl. .... 252/32.7 E; 252/46.6; 252/49.8; 252/59; 252/75; 252/78

[51] Int. Cl. .... C10m 3/42; C10m 3/40; C10m 3/32

[58] Field of Search..... 252/32.7 E, 49.8, 59, 78, 252/46.6, 75; 260/950

## [56] References Cited

## UNITED STATES PATENTS

|           |         |                       |            |
|-----------|---------|-----------------------|------------|
| 2,386,222 | 10/1945 | Lincoln et al. ....   | 252/45     |
| 2,577,636 | 12/1951 | Sperry.....           | 252/48.6   |
| 3,010,903 | 11/1961 | Clarke et al. ....    | 252/49.9   |
| 3,211,653 | 10/1965 | O'Halloran .....      | 252/50     |
| 3,410,801 | 11/1968 | Tunkel et al. ....    | 252/74     |
| 3,595,796 | 7/1971  | Duling et al. ....    | 252/73     |
| 3,825,495 | 7/1974  | Newingham et al. .... | 252/32.7 E |
| 3,843,534 | 10/1974 | Gates et al. ....     | 252/49.8   |

## OTHER PUBLICATIONS

Rounds, "Jour. Chemical & Engineering Data," Vol. 5, No. 4, (1960), pp. 499-507.

Primary Examiner—Delbert E. Gantz

Assistant Examiner—I. Vaughn

Attorney, Agent, or Firm—George L. Church; J. Edward Hess; Barry A. Bisson

## [57] ABSTRACT

An improved method of lubrication of a controlled-slip differential comprises using a lubricant comprising a static friction reducing amount of an aliphatic phosphate ester and a hydrocarbon base stock having a kinematic viscosity at 210°F. in the range of 1.5-200.0 c.s. and containing a major amount of a hydrogenated polymer of C<sub>5</sub>-C<sub>12</sub> olefin, such as a "true" isobutylene oligomer or of a blend of at least one C<sub>13</sub>-C<sub>29</sub> naphthene and from 0.1-20 parts by weight, based on said naphthene of at least one member from at least one of the following groups (a), (b), (c) and (d):

- a. a synthetic liquid C<sub>5</sub>-C<sub>8</sub> olefin homopolymer copolymer, or terpolymer;
- b. a member from group (a) above which is at least partially hydrogenated;
- c. a severely hydrorefined naphthenic lube containing less than 1% of gel aromatic hydrocarbons; and
- d. a severely hydrorefined paraffinic lube containing less than 1% of gel aromatic hydrocarbons; and wherein the amount of said blend which is present in said base stock is sufficient to provide a greater coefficient of traction, measured at 600 ft./min., 200°F., 400,000 p.s.i., than would be provided by substitution of the same amount of ASTM Oil No. 3 for said blend in said base stock. The preferred lubricant also contains an extreme pressure additive (e.g. tricresyl phosphate).

20 Claims, 4 Drawing Figures

PATENTED SEP 2 1975

3,903,001

SHEET 1 OF 4

FIGURE 1



CONTROLLED-SLIP DIFFERENTIAL

FIGURE 2  
"ROXANA LVFA" FRICTION VS. SLIDING SPEED



FIGURE 3  
"GENERAL MOTORS R-H" FRICTION TESTER DATA



FIGURE 4  
LVFA FRICTION VS. SLIDING SPEED



## LUBRICANT FOR A CONTROLLED-SLIP DIFFERENTIAL

## CROSS REFERENCE TO RELATED APPLICATIONS

The present application is related to the following listed United States applications,

| Serial No. | Filing Date                                         | Title/Inventor(s)                                                                                                                                                         | Serial No. | Filing Date                                        | Title/Inventor(s) |                                                                                                                                                                                                                                                                                                                                                                                           |
|------------|-----------------------------------------------------|---------------------------------------------------------------------------------------------------------------------------------------------------------------------------|------------|----------------------------------------------------|-------------------|-------------------------------------------------------------------------------------------------------------------------------------------------------------------------------------------------------------------------------------------------------------------------------------------------------------------------------------------------------------------------------------------|
| 621,443    | 3-8-67<br>(Now Abandoned)                           | Synthetic Lubricants from Low Molecular Weight Olefins - RICHARD S. STEARNS-IRL N. DULING DAVID S. GATES                                                                  | 5          | 80,779<br>(now U.S. 3,646,233<br>issued 2-29-72)   | 10-14-70          | and DAVID S. GATES                                                                                                                                                                                                                                                                                                                                                                        |
| 679,801    | 11-1-67<br>(Now U.S. 3,597,358,<br>issued 8-3-71)   | Traction Drive Transmission Containing Adamantane Compounds as Lubricant - IRL N. DULING-FREDERICK P. GLAZIER-DAVID S. GATES and ROBERT E. MOORE                          | 10         | 116,985<br>(now U.S. 3,825,495<br>issued 7-23-74)  | 2-19-71           | Reaction of Normal Paraffins with Adamantane Compounds - ROBERT E. MOORE                                                                                                                                                                                                                                                                                                                  |
| 679,833    | 11-1-67<br>(Now U.S. 3,595,796,<br>issued 7-27-71)  | Traction Drive Transmission Containing Naphthalenes, Branched Paraffins, or Blends of Naphthalenes and Branched Paraffins as Lubricant - IRL N. DULING and DAVID S. GATES | 15         | 133,637<br>(now U.S. 3,715,313<br>issued 2-6-73)   | 4-13-71           | Lubricant for Controlled-Slip Differential - THOMAS D. NEWINGHAM-ALEXANDER D. RECHUITTE-JOHN Q. GRIFFITH, III-MARCUS W. HASELTINE, JR.                                                                                                                                                                                                                                                    |
| 679,834    | 11-1-67<br>(Now U.S. 3,595,797,<br>issued 7-27-71)  | Blending Branched Paraffin Fluids for Use in Traction Drive Transmission - IRL N. DULING-DAVID S. GATES and MARCUS W. HASELTINE                                           | 20         | 135,295<br>(now U.S. 3,793,203<br>issued 2-19-74)  | 4-19-71           | Combination of Tractive Drive and Traction Fluid Comprising Saturated Cyclic Compounds - IRL N. DULING and FREDERICK P. GLAZIER                                                                                                                                                                                                                                                           |
| 679,851    | 11-1-67<br>(Now U.S. 3,598,740,<br>issued 8-10-71)  | Traction Drive Transmission Containing Paraffinic Oil as Lubricant - IRL N. DULING-DAVID S. GATES-THOMAS D. NEWINGHAM                                                     | 25         | 137,556<br>(now U.S. 3,793,203<br>issued 2-19-74)  | 4-26-71           | Chemical Reaction Products of Polyisobutylene - GARY L. DRISCOLL and MARCUS W. HASELTINE, JR.                                                                                                                                                                                                                                                                                             |
| 784,487    | 12-17-68<br>(now U.S. 3,646,224,<br>issued 2-29-72) | Conversion of Adamantane Hydrocarbons to Monooleins - ROBERT E. MOORE                                                                                                     | 30         | 144,165<br>(now U.S. 3,843,537<br>issued 10-22-74) | 5-17-71           | Chemical Reaction Product of Sulfur, Lard Oil and Polyisobutylene - ALEXANDER D. RECHUITTE-GRAY L. DRISCOLL                                                                                                                                                                                                                                                                               |
| 794,844    | 1-24-69<br>(Now U.S. 3,608,385,<br>issued 9-28-71)  | Friction Drive Fluid - IRL N. DULING and FREDERICK P. GLAZIER                                                                                                             | 35         | 152,303<br>(now U.S. 3,793,203<br>issued 2-19-74)  | 6-11-71           | Traction Transmission Containing Lubricant Comprising Gem-Structured Polar Compound - MARCUS W. HASELTINE, JR. and GARY L. DRISCOLL                                                                                                                                                                                                                                                       |
| 812,516    | 2-19-69<br>(Now U.S. 3,619,414,<br>issued 11-9-71)  | Catalytic Hydrofinishing of Petroleum Distillates in the Lubricating Oil Boiling Range - IVOR W. MILLS-MERRITT C. KIRK, JR. and ALBERT T. OLENZAK                         | 40         | 155,986<br>(now U.S. 3,843,537<br>issued 10-22-74) | 6-23-71           | Lubricant Comprising Gem-Structured Organo Compound - GARY L. DRISCOLL and MARCUS W. HASELTINE, JR.                                                                                                                                                                                                                                                                                       |
| 823,138    | 5-8-69<br>(Now U.S. 3,560,578,<br>issued 2-2-71)    | Reaction for Linking Nuclei of Adamantane Hydrocarbons - ABRAHAM SCHNEIDER                                                                                                | 45         | 162,773<br>(now U.S. 3,843,537<br>issued 10-22-74) | 7-15-71           | Blended Traction Fluid Containing Cyclic Compounds - IRL N. DULING and DAVID S. GATES                                                                                                                                                                                                                                                                                                     |
| 850,717    | 8-18-69<br>(now abandoned)                          | Hydrorefined Lube Oil and Process of Manufacture - IVOR W. MILLS and GLENN R. DIMELER                                                                                     | 50         | 162,896<br>(now U.S. 3,843,537<br>issued 10-22-74) | 7-15-71           | Method for Improving the Coefficient of Traction Using Hydrogenated Polymeric Styrenes-IRL N. DULING and DAVID S. GATES                                                                                                                                                                                                                                                                   |
| 876,993    | 11-14-69<br>(now U.S. 3,645,902,<br>issued 2-29-72) | Friction or Tractive Drive Fluid Comprising Adamantanes - IRL N. DULING-FREDERICK P. GLAZIER-DAVID S. GATES and ROBERT E. MOORE                                           | 55         | 163,543<br>(now U.S. 3,843,537<br>issued 10-22-74) | 7-15-71           | Blanched Olefin Polymers as Tractants - IRL N. DULING and DAVID S. GATES                                                                                                                                                                                                                                                                                                                  |
| 877,462    | 11-17-69<br>(now abandoned)                         | Combination of Traction Drive and Traction Fluid Comprising Saturated Cyclic Compounds - IRL N. DULING and FREDERICK P. GLAZIER                                           | 55         | 163,545<br>(now U.S. 3,843,537<br>issued 10-22-74) | 7-15-71           | C <sub>19</sub> -C <sub>29</sub> Naphthalenes as Tractants IRL N. DULING and DAVID S. GATES                                                                                                                                                                                                                                                                                               |
| 3,256      | 8-19-69<br>(now U.S. 3,648,531,<br>issued 3-14-72)  | Friction or Tractive Drive Fluid IRL N. DULING-FREDERICK P. GLAZIER-DAVID S. GATES and ROBERT E. MOORE                                                                    | 55         | 165,418<br>(now U.S. 3,843,537<br>issued 10-22-74) | 7-15-71           | Hydrorefined Naphthenic Oil as A Tractant - DAVID S. GATES and IRL N. DULING                                                                                                                                                                                                                                                                                                              |
| 28,942     | 4-15-70                                             | Process for Producing Polyisobutylene Oil - ALFRED E. HIRSCHLER and GARY L. DRISCOLL                                                                                      | 55         | 194,903<br>(abandoned 10-2-72)                     | 11-2-71           | Blended Traction Fluid Containing Hydrogenated Polyolefin - IRL N. DULING-DAVID S. GATES-FREDERICK P. GLAZIER-ROBERT E. MOORE-THOMAS D. NEWINGHAM                                                                                                                                                                                                                                         |
| 33,023     | 4-29-70<br>(now abandoned)                          | Combination of Tractive Drive and Traction Fluid Comprising Cyclic or Acyclic Compounds - IRL N. DULING and FREDERICK P. GLAZIER                                          | 60         |                                                    |                   | Combination of Tractive Drive and Traction Fluid Comprising Saturated Cyclic or Acyclic Compounds - IRL N. DULING and FREDERICK P. GLAZIER                                                                                                                                                                                                                                                |
| 52,301     | 7-6-70<br>(now U.S. 3,778,487<br>issued 12-11-73)   | Polyisobutylene Oil Having a High Viscosity Index - GARY L. DRISCOLL                                                                                                      | 60         |                                                    |                   | The disclosure of all of the above cited applications is hereby incorporated herein (by this reference). In particular, these applications disclose blended lubricants which are useful in the present invention, additives which can be useful in such lubricants and processes for making individual components of such blends.                                                         |
| 78,190     | 10-5-70<br>(now U.S. 3,737,477<br>issued 6-5-73)    | IRL N. DULING and DAVID S. GATES                                                                                                                                          | 60         |                                                    |                   | BACKGROUND OF THE INVENTION                                                                                                                                                                                                                                                                                                                                                               |
| 78,191     | 10-5-70<br>(now U.S. 3,676,521,<br>issued 7-11-72)  | Process of Preparing Synthetic Lubricants from Low Molecular Olefins - RICHARD S. STEARNS-IRL N. DULING and DAVID S. GATES                                                | 65         |                                                    |                   | As has been reported by R. L. Kostelak in <i>Lubrication</i> Vol. 56, No. 4, 1970 (pg. 49 et seq.), the principle of operation of the conventional differential in today's American automobile remains the same as the Pecqueur differential, invented in 1827. Although this "conventional differential" generally performs very satisfactorily, it has one serious shortcoming; namely, |

-Continued

"stalling," which occurs when either rear wheel loses traction. Due to the kinematics of the conventional differential design, the driving torque is divided equally between the two rear wheels and is limited by the wheel with the least traction. Hence, when one wheel loses traction, the vehicle does not move.

To prevent this shortcoming, engineers have developed many ingenious ideas and mechanisms. Each manufacturer has his own descriptive name for his particular mechanism; for example, Chevrolet Positraction, Chrysler Sure-Grip, and Ford Traction-Lok. Generally, however, a differential incorporating one of these mechanisms is called a "locking" or "limited slip" or "controlled-slip" differential.

The limited slip differential (sometimes referred to as "LSD") used in the American passenger car is essentially the same as a conventional differential except for the incorporation of some form of friction members (e.g. clutch plates or friction cones). The Kostelak article describes the conventional differential and typical controlled-slip differentials.

Another pertinent article is "Lubricants for Limited Slip Differentials" by John W. Allen, given at Fuels and Lubricants Meeting, Society of Automotive Engineers, Houston, Texas, Nov. 1-3, 1966.

Another description is found in U.S. Pat. No. 3,236,771 to H. J. Matson, issued Feb. 22, 1966. The Matson patent also describes some problems encountered in lubrication of an LSD.

#### SUMMARY OF THE INVENTION

In a combination of a controlled-slip differential and a lubricant therefor, an improvement comprises using a lubricant comprising a hydrocarbon base stock having a kinematic viscosity at 210°F. in the range of 1.5-200.0 c.s. and containing a hydrogenated "true" oligomer of isobutylene or a blend of at least one C<sub>13</sub>-C<sub>29</sub> naphthene and from 0.1-20 parts by weight, based on said naphthene, of at least one member from at least one of the following groups (a), (b), (c) and (d):

a. a synthetic liquid C<sub>5</sub>-C<sub>8</sub> olefin homopolymer (such as a "true" oligomer of isobutylene), copolymer, or terpolymer;

b. a member from group (a) above which is at least partially hydrogenated (preferably, to an iodine number less than 20, more preferably less than 5 and/or having a 195 UVA less than 2.0);

c. a severely hydrorefined naphthenic lube containing less than 1% of gel aromatic hydrocarbons; and

d. a severely hydrorefined paraffinic lube containing less than 1% of gel aromatic hydrocarbons;

and wherein the amount of said blend which is present in said base stock is sufficient to provide a greater coefficient of traction, measured at 600 ft./min., 200°F., 400,000 p.s.i., than would be provided by substitution of the same amount of ASTM Oil No. 3 for said blend in said base stock. The preferred lubricant has a viscosity in the range of 5-50 c.s. at 210°F., (typically 10-20 c.s.), has a channel point below 32°F. (more preferred below 10°F., typically 0° to -25°F.) and also contains an extreme pressure (EP) additive (e.g. tricresyl phosphate, zinc dithiophosphate, etc.) and an additive which lowers the static friction of the lubricant (e.g. a surface-active, organic phosphate ester of a linear aliphatic, ethoxylated alcohol).

Preferably, the C<sub>13</sub>-C<sub>29</sub> naphthene has a glass transition temperature in the range of -90° to -30°C. and contains as a structural nucleus, a cyclohexyl hydrindan, di(cyclohexyl) alkane, adamantane, spirodecane, spiropentane, perhydrofluorene, perhydrobiphenyl, perhydroterphenyl, decaline, norbornane, perhydroindacene, perhydrohomotetraphthene, perhydroacenaphthene, perhydrophenanthrene, perhydrocrysene, perhydroindane-1-spirocyclohexane, perhydrocarylophyllene, pinane, camphane, perhydrophenylnaphthalene or perhydropyrene.

These blended hydrocarbon base stocks are described in the aforementioned applications of Duling et al (e.g. see Ser. No. 33,023, filed Apr. 29, 1970) and in the application of Driscoll et al. The "true" oligomers of isobutylene are described in the applications of Driscoll et al).

One important property of an LSD lubricant is the relationship between the static coefficient of friction and the dynamic coefficients of friction at various sliding speeds. Generally, the required coefficients are for steel on steel; however, other reference materials can be used (e.g. steel on paper) depending on the mechanism to be lubricated.

The preferred methods for obtaining the required friction coefficients include two.

One is the "LVFA" (or Low Velocity Friction Apparatus) method. The LVFA method is described by T. D. Newingham in Publication 774A of the Society of Automotive Engineering (National Fluids and Lubricants Meeting, Tulsa, Oklahoma, Oct. 30-31, 1963)

The second method is the "R-H" method, which is described by M. L. Haviland et al, "Friction Characteristics of Controlled-Slip Differential Lubricants," pp 828-843, S. A. E. Transactions (1967).

Certain of the lubricants of the present invention, as will be further described hereinafter, produce unusual and very desirable friction curves when measured by either of these methods. These desirable curves can be described as "low static-high dynamic friction". A key component of these desirable lubricants is an effective amount of a surface-active organic phosphate ester of a linear aliphatic, ethoxylated alcohol, said amount (e.g. 0.1-10 wt%) being effective to reduce the static friction while not greatly reducing the dynamic friction.

#### BRIEF DESCRIPTION OF THE DRAWINGS

In the accompanying drawings, FIG. 1 is an illustration of a controlled-slip differential and will be referred to with reference to a test method for comparing the dynamic torque obtained from a given combination of lubricant and controlled-slip differential. The test can be useful in comparing various lubricants in a given differential.

For example, in a limited slip differential (LSD), the contact plates can be surfaced with swirl patterns to produce high friction. When the plate has become worn, the friction drops drastically and the LSD fails to perform any better than a conventional differential. With a high traction-LSD fluid, the friction property is inherent in the fluid itself and is not completely dependent on the patterned contact surfaces. Thus, the lubricated contacts can have high friction (or traction) even when badly worn.

With reference to FIG. 1, torque measurements are made by attaching a belt 10 around one of the rear wheels 8 and connecting the belt end to a calibrated

spring scale 11. The other rear wheel 1 is then turned by hand to slip the differential. The measurement when slip begins is taken as the "break-free torque". A second measurement is determined at approximately 40 rpm (with the wheel 1 being driven by a motor).

The differential in FIG. 1 consists of a ring gear 4, a differential pinion 6 and cross shaft, and a right 7 and a left 2 clutch plate attached to the differential case. The wheels are connected to the differential pinion by the right 5 and the left 3 side gears. Clutch plates are also attached to the left and right axle shafts. The differential assembly and the lubricant are contained in a housing 9.

FIGS. 2, 3 and 4 illustrate, for a number of lubricants, the relationship between the static coefficient of friction and the dynamic coefficient of friction at various sliding speeds. The FIGS. 2 and 4 data was obtained by the "LVFA" method; whereas, the FIG. 3 data was obtained by the "R-H" method.

#### EXAMPLE I

466 g. of a commercial  $\alpha$ -methyl styrene polymer, obtained by conventional acid-catalyzed polymerization, is placed in a 1-liter round bottomed flask, attached to a 1-inch column, and dry-distilled with essentially no reflux or fractionation at a pot temperature of about 290°C., and a vapor temperature of about 210°C. under a vacuum of about 6 millimeters of mercury. 373 g. of distillate are obtained and about 73 grams of material remain in the bottom of the flask at the end of the distillation. The commercial  $\alpha$ -methyl styrene polymer has a softening point of 210°F., a Gardner-Holdt viscosity of J-L, a specific gravity of 1.075, a refractive index at 20°C. of 1.61, a molecular weight of 685, an iodine number of 0, an acid number of 0, and a saponification number of 0.

#### EXAMPLE II

300 g. of the distillation product of Example I is placed in a 316 stainless steel bomb along with 7.5 grams of Raney nickel catalyst and the bomb is pressurized to 3,000 p.s.i.g. of 100% hydrogen while heat is applied until the temperature in the bomb is 150°C. At that point an exothermic reaction occurs and heating is discontinued. The temperature is allowed to rise to about 230°C. and the hydrogen pressure is maintained at 3,000 p.s.i. for 6 hours at which time the bomb is slowly cooled to ambient temperature while maintaining the hydrogen pressure at 3,000 p.s.i. in order to avoid dehydrogenation of the hydrogenated product. The resulting perhydrogenated poly ( $\alpha$ -methyl styrene) oil is topped to remove components boiling below 125°C. The remaining perhydrogenated naphthene product has a KV210 of 11.07 c.s. and a KV100°F. of 327.8 c.s. Analysis by nuclear magnetic resonance (NMR) shows the oil of this example to contain about 40% of trimers (mostly hydrindan form), and 60% dimers, mainly 1,1,3-trimethyl-3-cyclohexyl hydrindan.

#### EXAMPLE III

A blend of two commercially available polybutene polymers (i.e., 90 vol.% Indapol L-100 and 10% Oronite Special 6) is completely hydrogenated to produce a hydrogenated polybutene oil which analyzes 0.5 mole percent olefin by the ultraviolet absorbence method. The hydrogenation is at 200°C., 2,000 p.s.i. of 100% hydrogen for 6 hours using Harshaw NI0104P catalyst.

The resulting hydrogenated polyolefin oil has a KV210°F. of 13.54 c.s. and a KV100 of 162.8.

#### EXAMPLE IV

5 A blended base oil was compounded from 61.0 volumes of the naphthene product of Example II and 33.1 volumes of the hydrogenated polyolefin oil of Example III. Then 5.9 volumes of a commercial "limited slip axle additive" (Lubrizol Company, Anglamol 99LS) was 10 added to the blend to produce a formulated lubricant. Table 1 describes typical properties of Anglamol 99LS.

TABLE 1

|                                      |         |
|--------------------------------------|---------|
| Specific Gravity at 60°F., (15.6°C.) | 1.055   |
| Pounds per Gallon at 60°F., U.S.     | 8.79    |
| Pounds per Gallon at 60°F., IMP.     | 10.55   |
| Viscosity at 210°F., (98.9°C.) SUS   | 60      |
| Viscosity at 210°F., cSt.            | 10.2    |
| Weight Percent of:                   |         |
|                                      | Typical |
| Sulfur                               | 29.2    |
| Phosphorous                          | 2.0     |

25 Similarly, other blended base oils (e.g. comprising synthetic paraffins and naphthenes) and other gear oil additives can be used to formulate such lubricants. Other useful additives are those mentioned by F. G. Rounds, *Journal of Chem. and Eng. Data*, Vol 5, No. 4, October, 1960, pp. 504-505. Useful blended base oils 30 and additives are disclosed, for example, in previously cited applications Ser. Nos. 33,023, and 52,301.

#### EXAMPLE V

35 Another useful lubricant for a controlled-slip differential, and which is also useful for lubrication of a traction drive transmission, comprises a blend of the following (all hydrogenations are to at least 98% saturation):

|    | VOLUME | COMPONENT                          | KV210°F.<br>(c.s.) | KV100°F.<br>(c.s.) |
|----|--------|------------------------------------|--------------------|--------------------|
| 45 | 7.0    | Hydrogenated Cosden SH06           |                    |                    |
|    | 28.0   | Polybutene                         | 11.04              | 124                |
|    | 31.6   | Hydrogenated Cosden SH15           | 33.5               | 744                |
| 50 | 21.0   | Polybutene                         | 23                 | 2463               |
|    | 7.4    | Hydrogenated Poly $\alpha$ -Methyl | 4.65               | 39.6               |
|    | 3.0    | Styrene                            |                    |                    |
|    | 1.0    | Hydrogenated Poly $\alpha$ -Methyl |                    |                    |
|    | 1.0    | Styrene                            |                    |                    |
|    | 1.0    | Anglamol 93 (E.P. Additive         |                    |                    |
|    | 1.0    | Amoco 9000 (Dispersant)            |                    |                    |
|    | 1.0    | Ultraphos 11 (Low Static           |                    |                    |
|    | 1.0    | Modifier)                          |                    |                    |
|    | 1.0    | Synthetic Sulfurized Oil           |                    |                    |

55 The use in this lubricant of high and low viscosity fractions of the naphthene and paraffin is an example of "dumbbell-blending" to improve viscosity index.

The Ultraphos 11 additive is a surface-active, organic phosphate ester of a linear aliphatic, ethoxylated alcohol, and is further described hereinafter.

60 The synthetic sulfurized oil is the invention of Alexander D. Recchuiti and is the subject of application Ser. No. 135,466 (now abandoned). This oil can be used as a replacement for sulfurized sperm oil and can be made by heating sulfur and a blend of from 30-95% lard oil and 70-5% of one or a mixture of  $C_{12}$ - $C_{24}$  acyclic monoolefin. For example, 10 weight percent of sulfur was added at 250°F. to 90 weight percent of a blend

of 85 volumes of lard oil (No. 1 grade) and 15 volumes Chevron C<sub>15</sub>–C<sub>20</sub>  $\alpha$ -olefin. The sulfur-containing mixture was heated to 375°F. and maintained at that temperature, with stirring, for 2 hours, then cooled to 200°F., and, finally, blown with air for 1 hour.

Another procedure for making the synthetic sulfurized oil is to heat the lard oil-olefin blend to about 300°F., add sulfur (e.g. 5–25%) over a 30 minute period (with agitation), then bring the temperature to 335°F., maintain for 2 hours, cool to 200°F. and finally blow with air for 16 hours. This latter procedure was used for the synthetic sulfurized oil in the above listed lubricant.

The channel point of a lubricant is determined by drawing a channel with a spatula in a sample of lubricant, at a given temperature, and finding the maximum temperature where the walls of the channel no longer cave-in.

#### EXAMPLE VI

A well-worn limited slip differential in a 1965 Buick Skylark (driven over 65,000 miles) was used to compare lubricants, by the previously described method.

The used, original fill fluid was replaced with a fresh conventional petroleum-based LSD fluid (e.g. solvent refined paraffinic lube plus Anglamol 99LS). Torque measurements were made periodically for the next 500 miles. For the last 100 miles, a 6 p.s.i. difference in air pressure in the rear tires caused the differential to slip constantly. It was believed that this tire pressure difference caused the fresh fluid to work into the contact areas. At the end of 500 miles, the conventional fluid was replaced with the blended "traction-LSD fluid" of Example IV, which had the same viscosity at 100°F. and the same additive system as the petroleum-LSD fluid. After 40 miles of driving with the 6 p.s.i. air pressure differential in the rear tires the torque measurement at the low speed dynamic conditions was nearly double that observed when the petroleum-LSD fluid was used. There was little difference in the break-free torque since the static friction is primarily dependent on the

additive system. Table 2 presents the test data obtained from this testing.

TABLE 2

| 5  | Fluid                       | Torque Through Worn Limited Slip Differential |            |        |
|----|-----------------------------|-----------------------------------------------|------------|--------|
|    |                             | Odome-<br>ter                                 | Break-Free | 40 rpm |
| 10 | Original Fill               | 66055                                         | 80         | 13     |
|    | Petroleum-LSD Fluid charged | 66070                                         | —          | —      |
|    |                             | 66070                                         | 85         | 13     |
|    |                             | 66104                                         | 80         | 12.5   |
|    |                             | 66400                                         | 92         | 12     |
|    | Traction-LSD Fluid charged  | 66509                                         | —          | —      |
| 15 |                             | 66541                                         | 90         | 23     |
|    |                             | 66650                                         | 90         | 26     |
|    |                             | 69207                                         | 95         | 25     |

A graphic representation of the results of this testing can be found in "Design and Development of Fluids for Traction and Friction Type Transmissions," by M. W. Haseltine, Jr. I. N. Duling, P. E. Hagstrom, R. J. Stenger and J. S. Gates, Society of Automotive Engineers Publication 710937 (Meeting Oct. 26–29, 1971, St. Louis, Mo.)

25 The high dynamic friction also helped reduce chatter. With high dynamic friction, static friction can increase to a higher level before chatter will occur. Thus, low static modifying additives are effective for a longer period of time in a high traction-LSD fluid. This results in longer LSD fluid life before chatter occurs. In the present invention a preferred low static friction modifier is 0.1–10% of a surface-active organic phosphate ester of a linear, aliphatic ethoxylated alcohol.

#### EXAMPLE VII

Conventional petroleum-LSD lubricant and the blended "Traction-LSD" lubricant of Example IV were compared in four limited slip differentials, by the previously described test method. The results of these tests are summarized in Table 3. The performance of each differential was improved when lubricated by the blended traction-LSD lubricant.

TABLE 3

| Car             | Fluid         | Torque Through Various Limited Slip Differentials |                            |        | Odome-<br>ter<br>at<br>Fluid<br>Change |
|-----------------|---------------|---------------------------------------------------|----------------------------|--------|----------------------------------------|
|                 |               | Odometer at<br>Torque Test                        | Torque, lbs.<br>Break-Free | 40 RPM |                                        |
| Chev.<br>1969   | Original      | 11151                                             | 20                         | 10     | 11151                                  |
|                 | Petroleum-LSD | 11437                                             | 22–23                      | 12–14  | 11437                                  |
|                 | Traction-LSD  | 11449                                             | 25                         | 15–20  |                                        |
|                 |               | 11539                                             | 20                         | 21–22  |                                        |
| Chev.<br>1969   | Original      | 12808                                             | 22–25                      | 6–9    | 12808                                  |
|                 | Petroleum-LSD | 13239                                             | 20–25                      | 6–7    | 13239                                  |
|                 | Traction-LSD  | 13274                                             | 20                         | 12–14  |                                        |
|                 |               | 13309                                             | 20                         | 12–14  |                                        |
|                 |               | 13762                                             | 19                         | 10–12  |                                        |
| Pontiac<br>1970 | Original      | 05721                                             | 30                         | 21–23  | 05721                                  |
|                 | Petroleum-LSD | 06578                                             | 30–32                      | 20     | 06578                                  |
|                 | Traction-LSD  | 06823                                             | 35                         | 28–29  |                                        |
|                 |               | 06981                                             | 35                         | 30     |                                        |
| Ford            | Original      | 18617                                             | 90                         | 20     | 18617                                  |
|                 | Petroleum-LSD | 19145                                             | 80–90                      | 22     | 19145                                  |
|                 | Traction-LSD  | 19198                                             | 75                         | 40     |                                        |
|                 |               | 19244                                             | 75                         | 40     |                                        |

Any of the usual gear lube additives can be used in the lubricant-differential combination of the present invention; however, especially beneficial results are obtained when 0.25-10% (based on the base stock) Ultraphos 11 (or less preferred, Ultraphos 12) is used as one of the additives. Ultraphos 11 is marketed by Witco Chemical Company and has the following typical properties:

$KV_{210} = 23.44$  c.s.  
 $KV_{100} = 217.20$  c.s.

Melting Point = 0°C.

Glass Transition Temperature = -62°C.

Elemental Analysis

|             |                  |
|-------------|------------------|
| Carbon      | 58.16%           |
| Hydrogen    | 10.47%           |
| Oxygen      | 20.44%           |
| Ash         | 1.58%            |
| Phosphorous | 5.77%            |
| Sulfur      | 0.4% (Schoniger) |
| Nitrogen    | <0.10%           |
| Chlorine    | <10 ppm          |

ASTM-VI = 142  
 VTF-VI = 132

Alternatively, Antara LB400 (General Aniline and Film) can be used instead of Ultraphos as a low static modifier.

Another useful multipurpose additive package which is useful in such lubricants is 2-15% Anglamol 93, which has been previously described and which is a product of Lubrizol Company and comprises a mixture of zinc phosphorodithioate and chlorinated hydrocarbons, a typical analysis being 3% Zn, 3% P, 16.5% Cl and 16.0% S. A useful extreme pressure additive can consist essentially of tricresyl phosphate, or a zinc dialkyl dithiophosphate, or a mixture thereof.

The present invention involves novel compositions which contain chemical reaction products which can be produced by the action of sulfur or sulfur monochloride on lard oil and the polyolefins or polyolefin oils of the aforementioned application Ser. No. 52,301. Such cosulfurized compositions are described in copending application Ser. No. 137,556 and are useful as lubricant additives, particularly in lubricants for tractive drives and limited slip differentials, and are generally useful as a replacement for sulfurized sperm oil.

A novel substitute for sulfurized sperm oil can be obtained by sulfurizing a blend of 90 to 30 parts by weight of lard oil and 10 to 70 parts of an olefin containing 12 to 128 carbon atoms. The sulfurization is carried out using elemental sulfur. Sulfur monochloride can be used for both sulfurizing and chlorinating simultaneously. The sulfurization involves cooking at from 330° to 445°F. for 20 minutes to 10 hours followed by blowing with a gas (preferably, at from 125° to 340°F. for 30 minutes to 20 hours) to remove hydrogen sulfide. With sulfur monochloride, the preferred cooking temperature is in the range of 150-250 (under pressure if desired). The sulfurized oils can contain from 5 to 25 weight percent sulfur as based on the blend of olefin and lard oil (i.e., 5 to 25 parts by weight of sulfur, per 100 parts by weight of olefin-lard oil blend).

For example, one embodiment of the invention involves using the previously described lubricants and from 0.1-10% of a composition consisting essentially of a sulfur-containing chemical reaction product of a mixture of lard oil and a "true" isobutylene oligomer, that is, a branched olefin hydrocarbon having 4N carbon

atoms where N is an integer from 3-32, said olefin hydrocarbon having the formula:



10

wherein n is an integer from 0 to 29 inclusive, and wherein Z is:



or



or



or



or



For example, in tetraisobutylene, for one isomer, n is 1 and Z is (D); for another, n is 2 and Z is (B); for another n is 2 and Z is (A); for another, n is 1 and Z is (C); for another n is 1 and Z is (E). For triisobutylene, for one isomer, n is 0 and Z is (D); for another, n is 0 and Z is (C) or (E); for another, n is 1 and Z is (A); and for another n is 1 and Z is (B).

40

45

50

55

60

65

The sulfurized product can be produced by blending from 90 to 30 parts of lard oil and from 10 to 70 parts of polyisobutylene, sulfurizing the blend and then blowing the co-sulfurized blend (or co-reaction product) with a gas to remove hydrogen sulfide. The lard oil and olefin generally are blended together at from 65°F. to 340°F. and the sulfur added while the blend is within this temperature range. In general, the preferred process conditions are those taught in application Ser. No. 135,466 of Rechuite, filed on Apr. 19, 1971.

The preferred commercial lard oil generally is described as winter grade lard oil. The principal difference between the less preferred grades such as No. 1 lard oil and the preferred grade is in the greater amount of saturated free fatty acids present in the less preferred grades, which can reduce the solubility of the product. The polyisobutylene, suitable for use in the present invention, can contain from 12 to 40 carbon atoms, preferably from 12 to 24 carbon atoms, more preferred 16 or 20. The amount of sulfur generally varies from about 5 to 25 percent by weight as based on the blend of lard oil and polyisobutylene. An "inactive" sulfurized product is generally desired; therefore, the preferred oils can contain from 6 to 11 percent as based on said

blend. Under the reaction conditions specified herein, this amount of sulfur will become chemically bonded in an inactive form. The resultant product containing 6 to 11 percent sulfur, as based on the blend of lard oil and polyisobutylene, is useful as a friction modifier for many applications as well as a cutting oil

The amount of sulfur in a given sample of oil is readily determined by X-ray fluorescence. After the amount of total sulfur is determined 100 g. of the oil sample and 20 g of copper powder are placed in a tall 250 ml. beaker set up on a hot plate and equipped with a thermometer and an Unger stirrer operated at 1,750 rpm. The sample is heated to 350°F. within a 5 minute period and maintained at 350°± 5°F. for 1 hour after which it is cooled and filtered through filter paper to remove the copper powder. The sulfur content of the sample is again determined by X-ray fluorescence which is the inactive sulfur. The loss of sulfur (total minus inactive sulfur) is the amount of active sulfur in the original. The amount of active sulfur in the sulfurized oil being used as a friction modifier should be less than about 2.5%. Generally the preferred friction modifiers which contain 6-11% total sulfur will also contain from 1 to 2% active sulfur.

After cooking the sulfurized oil is blown with a gas to remove H<sub>2</sub>S. Any gas may be used which dissolves (or otherwise removes) H<sub>2</sub>S and does not significantly react with the sulfurized oil. Suitable gases include air, nitrogen, carbon dioxide and gaseous perhalogenated hydrocarbons. Air is preferred for obvious economic considerations. The blowing is most simply carried out by bubbling the gas through the sulfurized oil. Alternatively the oil may be sprayed into the gas or a falling curtain of the oil in the gas may be used. Generally the blowing is carried out at from 125° to 340°F. In the case of the sulfurized oils containing minimal active sulfur the blowing should not be carried out above about 250°F. when air is the gas. When a high sulfur content (16-30%) oil is being made it is preferred to use gas blowing temperatures above 190°F. as this minimizes the active sulfur lost in processing.

The sulfur may be added either as elemental sulfur or sulfur monochloride (S<sub>2</sub>Cl<sub>2</sub>). The elemental sulfur is usually preferred for the low sulfur (6-11%) oils but S<sub>2</sub>Cl<sub>2</sub> is often preferred for the cutting oil applications because the chlorine also reacts with the oil and serves to improve the antiweld characteristics of the product.

The sulfurized oils described above are useful as friction modifiers in fluids of the present invention to reduce the static friction more than the dynamic friction. Generally, in such fluids the sulfurized oils are used at from 0.5 to 10%, typically 1-5%, of the overall fluid.

#### EXAMPLE VIII

A three necked, 1-liter, round-bottomed flask was equipped with a mechanical stirrer, a gas inlet tube (which also serves for intermittent product removal), and a reflux condenser containing a thermometer which dipped into the liquid layer and was capped with a gas exit tube leading through a mercury bubbler to the atmosphere. Nitromethane (200 ml.) and stannic chloride (5 ml. = 11.15 g.) were added to the flask and the isobutylene flow started. The reaction was maintained at 30°± 1°C. with an ice bath. The rate of isobutylene addition was 7.2 g/min. which resulted in 8.5 ml/min. of product (density~0.85) formation. At 20 min. intervals, the isobutylene feed and the stirrer were

stopped and the layers permitted to separate. The top oil layer (170 ml.) was removed and the nitromethane (bottom) layer was returned to the reactor with 5 ml. (3% of product volume) fresh nitromethane added to compensate for solubility losses. After four twenty-minute runs, the reaction was stopped. The catalyst in the nitromethane layer was readily killed with water with some production of HCl fumes. No difficulty with an exotherm was encountered when killing the catalyst.

10 The combined oil layers (665 ml. including 20 ml. nitromethane) were washed with water, with 5% sodium hydroxide solution, and twice more with water. A solvent such as pentane or hexane can be added to facilitate handling.

15 Although the oil of this example contains all of the novel polyisobutylene oligomers in the series C<sub>16</sub>-C<sub>20</sub>.C<sub>48</sub>+, fractional vacuum distillation can be used to obtain fractions relatively pure in a given oligomer (e.g. C<sub>16</sub> or "tetraisobutylene").

20 In the reaction of this example, small amounts of water in the catalyst and/or feed material can act as a reaction promoter. If extremely pure materials are used in the process, a small amount of water can be added to initiate or hasten the reaction. A lower alcohol (e.g., methanol) or acid (e.g., acetic acid) can also be used as such a promoter. Generally, the reaction rate can be increased (over anhydrous) by addition of 0.1-1.5 moles H<sub>2</sub>O per mole of SnCl<sub>4</sub>.

25 Polyolefin products, such as that of this example, can contain residual tin and chlorine (e.g., 250-5,000 ppm Cl). These elements, particularly the tin, can be present as a metal-organic compound which imparts EP (extreme pressure lubricant) properties to the product. However, if one desires, the chlorine (e.g., 2,000 ppm) can be removed from the product by heating the product with calcium oxide (lime) followed by filtration. Mild catalytic hydrogen treatment (e.g. 200 psi. of H<sub>2</sub>,200°C., Harshaw NI-0104P catalyst) can also be used to reduce the tin and chlorine content to very low levels (e.g., Cl from 2,000 ppm. to 6 ppm) and the resulting polyisobutylene (which can be present with hydrogenated polyisobutylene) can be used to produce the sulfurized product of the present invention.

45

#### EXAMPLE IX

30 Polyisobutylene oil, produced as in Example I, was fractionally distilled, at atmospheric pressure, to obtain a product which contained at least 80 weight percent of the C<sub>16</sub> isobutylene oligimer (i.e., "tetraisobutylene"). The predominantly C<sub>16</sub> fraction boiled in the range of 190°-245°C. and over 90 volume percent boiled at 240°C. Analysis by vapor phase chromatography showed that this predominantly C<sub>16</sub> fraction contained less than 10 weight percent C<sub>12</sub> oligimer and less than 10 weight percent of the C<sub>20</sub> and higher oligimers.

55

#### EXAMPLE X

60 Twenty-two hundred and sixty ml. of winter strained lard oil were blended with 400 ml. of tetraisobutylene (prepared as in Example 3) in a 5 L kettle equipped with a vibromixer. The mixture was heated to 250°F. and the vibromixer operated at maximum speed. Sulfur (239 g) was added and the temperature of the mixture raised to 375°F. for 2 hours. The mixture was then cooled to 200°F. and air was bubbled through the mixture by means of a glass tube at a moderate rate (below that at which splashing and agitation take place) for

65

one hour. The resulting sulfurized oil was analyzed and found to contain 8.23% sulfur. A ten gram portion of the sulfurized oil was dissolved in 100 g. of a commercially available solvent refined paraffinic lube having a viscosity at 210°F. of 40.45 SUS, an ASTM viscosity index of 104 and containing 12% aromatics (by ASTM D2007). The oil solution remained clear with no separation after being tested at 36°F. overnight and for one week at room temperature.

Similarly, lubricants can be compounded comprising a synthetic sulfurized oil and/or a surface active, organic phosphate ester of a linear aliphatic ethoxylated alcohol and various hydrogenated fractions of "true" polyisobutylene (or of other acyclic polyolefin oils). Properties of some such "true" polyisobutylene oils are summarized below (for comparison, properties of petroleum lubes are included) in Table 4.

Table 4

| COMPARISON OF LPIB* WITH PETROLEUM BASE OILS |         |          |          |           | Pour Pt<br>°F | Flash<br>°F |
|----------------------------------------------|---------|----------|----------|-----------|---------------|-------------|
|                                              | ASTM VI | KV/210°F | KV/100°F | SUS/100°F | KV/0°F        |             |
| LPIB                                         | 115     | 1.54     | 4.37     | 40.3      |               |             |
| HLPIB**                                      | 118     | 1.35     | 3.53     | 37.7      | 20.1          | <-75 155    |
| naphthenic oil                               | 52      | 1.39     | 4.27     | 40.0      | 36.9          | -90 225     |
| LPIB                                         | 100     | 2.39     | 8.78     | 54.6      |               | 235         |
| HLPIB                                        | 102     | 2.47     | 9.21     | 56.2      | 139           | <-70 255    |
| naphthenic oil                               | 31      | 2.26     | 9.53     | 57        | 212           | -70 295     |
| paraffinic lube                              | 98      | 2.63     | 10.28    | 60        | 163           | 0 345       |
| LPIB                                         | 98      | 4.46     | 24.9     | 119       |               | 305         |
| HLPIB                                        | 100     | 4.20     | 22.3     | 108       | 810           | <-75 315    |
| naphthenic oil                               | <0      | 3.60     | 22.9     | 110       | 1730          | -45 320     |
| hydrogenated naphthenic oil                  | 7       | 3.60     | 22.0     | 106       | 1330          | -50 325     |
| paraffinic lube                              | 104     | 4.27     | 22.9     | 110       | 747           | 0 385       |
| HLPIB                                        | 96      | 7.17     | 55.3     | 256       | 3,650         | <-50 380    |
| naphthenic oil                               | 2       | 5.63     | 54.9     | 255       | 12,500        | <-25 350    |
| paraffinic lube                              | 103     | 7.36     | 55.1     | 256       | 3,860         | 0 450       |
| HLPIB                                        | 88      | 11.70    | 124.1    | 574       | 11,810        | <-50 415    |
| naphthenic oil                               | <0      | 8.55     | 128.4    | 595       | 94,400        | -10 390     |
| hydrogenated naphthenic oil                  | <0      | 8.52     | 127.0    | 588       | 91,000        | -5 390      |
| paraffinic bright stock                      | 97      | 12.38    | 126.1    | 584       | 16,300        | 0 495       |

\*Linear "true" Polyisobutylene Oil (Unhydrogenated).

\*\*Fully Hydrogenated "true" Linear Polyisobutylene (hydrogenation with Ni on Kieselguhr, 1000 psi H<sub>2</sub>, 400°F).

### EXAMPLE XI

Winter strained lard oil (2,525 ml.) was blended with 450 ml of 80+% pure triisobutylene (prepared by a distillation similar to that used in Example 6 but at a lower temperature), in a 5 L kettle equipped with a vibromixer. The mixture was heated to 250°F. and the vibromixer operated at maximum speed. These conditions were maintained while 266 g. of sulfur were added over a period of 30 minutes. The temperature was raised to 375°F. for 2 hours. The mixture was then cooled to 200°F. for 1 hour and air was bubbled through the mixture by means of a glass tube at a moderate rate below that at which splashing takes place. The resulting sulfurized oil was analyzed and found to contain 8.5% sulfur as based on the total composition. A 10 gram portion of the sulfurized oil was dissolved in 100 g. of the solvent refined paraffinic lube described in example X. The oil solution remained clear with no separation after being tested at 36°F. overnight and for 1 week at room temperature.

### EXAMPLE XII

A useful lubricant for a controlled-slip differential, and which is also useful for lubrication of a traction drive transmission, comprises a blend of the following (the hydrogenation was to at least 98% saturation):

Parts  
by Volume

|      |                                       |
|------|---------------------------------------|
| 86.6 | hydrogenated "true" polyisobutylene*  |
| 7.4  | Anglamol 93                           |
| 3.0  | Amoco 9000                            |
| 2.0  | Ultraphos 11                          |
| 1.0  | synthetic sulfurized oil of Example X |

\*Made by hydrogenation of a 12.0 c.s. (at 210°F.) distillate fraction of the product of Example VIII.

35 Compared with the naphthenic distillates and hydrogenated naphthenic oils the polymer oils have much higher viscosity indexes and much lower 0°F viscosities and pour points, especially in the more viscous cuts. The pour points for the linear polyisobutylenes are much lower than for the solvent refined paraffinic oils 40 while the viscosity characteristics of the two are quite similar. Flash points for the LPIB oils are lower. This may be caused by improper distillation.

45

### EXAMPLE XIII

Friction data was obtained for a number of oils. The friction data was used to plot the curves in FIGS. 2, 3 and 4 hereof. The data for FIGS. 2 and 4 were obtained 50 by the LVFA method (using the apparatus marketed by Roxana Machine Works, St. Louis, Missouri). The data for FIG. 3 was obtained by the R-H Friction method, using the General Motors Corporation apparatus.

The following Table identifies the oils of FIGS. 2, 3 and 4:

| Oil No. |                                                       |
|---------|-------------------------------------------------------|
| 60      | 1 The blended hydrocarbon portion of Oil 4            |
|         | 2 Oil 1 plus 1 vol % Ultraphos 11                     |
|         | 3 Oil 1 plus additives *                              |
|         | 4** Oil 3 plus 1 vol. % Ultraphos 11                  |
|         | 5 Commercial Petroleum base LSD fluid (Texaco TL3450) |
| 65      | 6 Hydrogenated true polyisobutylene                   |
|         | 7 Oil 6 plus 1 vol. % Ultraphos 11                    |
|         | 8 Oil 6 plus 5 vol. % Ultraphos II                    |

\*The additives are those of the lubricant of Example V, excepting the Ultraphos 11.

\*\*Oil 4 is the lubricant of Example V

The curve for Oil 1 in FIG. 2 shows that the blended hydrocarbon base oil used in the lubricant of Example V had a higher static friction than the dynamic friction at sliding speeds in the range of about 20-120 feet per minute. The blended base oil of Example V was a blend of naphthenes (i.e., hydrogenated  $\alpha$ -methyl styrene oligomers) and hydrogenated polyolefins (i.e., polybutenes).

The curve for Oil 2 in FIG. 2 shows that the Ultra-phos 11 (a surface active phosphate ester of a linear aliphatic ethoxylated alcohol) produced a lowered static friction in the blended naphthene-hydrogenated polyolefin hydrocarbon base oil, without greatly altering the average dynamic friction.

Similarly, the curves for Oils 3 and 4 establish that the other additives in the lubricant of Example V did not appreciably lower the static friction but that the phosphate ester additive (Ultra-phos 11) produced the low static friction in the lubricant.

The friction curve for Oil 5 of FIG. 2 is that of a conventional commercial prior art lubricant (containing a petroleum base oil) for a limited slip differential. The curve for Oil 5 shows that this prior art lubricant has a much higher static friction than the average dynamic friction in the 20-120 feet per minute range of sliding speed.

The curves of FIG. 3 show that similarly shaped curves, to those of FIG. 2, are obtained by the "R-H" method.

The curves of FIG. 4 show that the phosphate ester additive can be used to lower the static friction, without greatly altering the dynamic friction in hydrogenated polyolefin oils, particularly oils consisting essentially of hydrogenated "true" polyisobutylene. The hydrogenated polyisobutylene used in Oils 6, 7 and 8 had a viscosity at 210°F of 33.5 c.s. (158 SUS) and at 100°F. of 742 c.s. (3,440 SUS).

The curves for Oils 7 and 8 of FIG. 4, indicate that a lubricant containing a major portion of a hydrogenated polybutene oil (especially a "true" polyisobutylene) and the phosphate ester in amount effective to lower the static friction can be useful as a lubricant for a limited slip differential. Other, conventional lube oil additives, e.g., antiwear, dispersant, antirust, antifoam, extreme pressure (EP), and oxidation inhibitors, can also be added to such a lubricant.

Other uses for a lubricant containing the phosphate ester and the hydrogenated polybutylene oil are in wet clutches (such as are marketed by Borg Warner for heavy duty trucks) and in wet brakes (as those used in tractors). For wet clutches and brakes a lower viscosity oil (e.g., 40-500 SUS at 100°F.) is generally desirable.

Other useful additives (instead of or with Ultra-phos 11) are Antara LB400 and Ortholeum 162. The lubricants containing the Ortholeum 162 have the better heat stability (that is, to maintain low static friction) after 100 hours aging at 300°F. Ortholeum 162 consists essentially of dilauryl phosphate and other similar mixed alkyl acid orthophosphates. Other useful phosphate ester additives (to lower static friction) are the phosphate esters of ethoxylated aromatic hydroxy compounds and their mixed esters with aliphatic hydroxy compounds. The esters can be part esters, (which produce an acidic pH in water, (e.g., pH about 2).

The blended fluids and limited slip differential lubricants referred to herein, especially that of Example IV, can be used to increase traction between two rolling el-

ements. When traction fluid is used to lubricate high speed ball bearings - for an example, the main shaft bearings in a turbine engine - it reduces ball skidding. Ball skidding is one of the factors limiting shaft speed.

Accordingly, such lubricants can be used for high speed and highly loaded bearings. They can also be used for lubrication of overrunning clutches. Such lubricants (in the appropriate viscosity range) can also be useful in conventional nontraction type automotive transmissions to provide improved lock-up and provide for the use of fewer clutch plates. Furthermore, a coating, generally paper, asbestos or resin, is used on clutch plates to increase the coefficient of friction between the plates. This plate coating can sometimes be eliminated when using the fluids of the present invention in such a transmission.

During engagement, there is a sliding motion between the cam or rollers and the races in overrunning clutches. Since wear occurs during the engagement period, a lubricant which reduces engagement time will reduce wear and extend service life. In one test, engagement was reduced from 11 to two revolutions simply by replacing the conventional petroleum oil grease with a grease component of a naphthene-paraffin blend similar to that of Example IV. The traction fluid and its grease show the greatest advantage in clutches where load is high enough to elastically deform the rollers or cams.

Unless otherwise specified, all percentages herein are by weight.

An especially useful naphthene component of a blended LSD FLUID (as in Example V) is 4,9-cis-1-cyclohexyl-1,3,3-trimethylhydrindane, which can be prepared in high yield (about 90%) by the hydrogenation of 1-phenyl-1,3,3-trimethylindane over a catalyst containing nickel, palladium or rhodium, in which the hydrogen pressure is held in the range of 600 to 1,500 psig, and the temperature is held substantially in the range of 200°C to 225°C. This process is the invention of Peter Hosler and David S. Gates and is claimed in a later filed application, Ser. No. 218,338, Jan. 17, 1972.

The invention claimed is:

1. A lubricant composition comprising a phosphate ester or mixture of esters selected from a surface active organic phosphate ester of a linear aliphatic ethoxylated alcohol or a mixed alkyl acid orthophosphate and a hydrocarbon base stock having a kinematic viscosity at 210°F in the range of 1.5-200.0 c.s. and comprising a major amount of (A) hydrogenated liquid polymer of  $C_3-C_{12}$  olefin or of (B) a blend of at least one  $C_{13}-C_{29}$  naphthene and from 0.1-20 parts by weight, based on said naphthene of at least one member from at least one of the following groups (a), (b), (c) and (d):

- a liquid  $C_3-C_8$  olefin homopolymer, copolymer, or terpolymer;
- a member from group (a) above which is at least partially hydrogenated;
- a severely hydrorefined naphthenic lube containing less than 1% of gel aromatic hydrocarbons; and
- a severely hydrorefined paraffinic lube containing less than 1% of gel aromatic hydrocarbons;

and wherein the amount of said phosphate ester or mixture which is present in said composition is effective to reduce the static friction, measured by the low velocity friction apparatus, of said base stock.

2. The composition of claim 1 and containing in the range of 0.1-10% by weight of said phosphate ester or mixture.

3. The composition of claim 1 wherein said major amount is of a true oligomer of isobutylene.

4. The composition of claim 1 wherein said hydrogenated polymer of component (a) and said hydrogenated polymer of component (b) are at least 80 mole percent saturated.

5. The composition of claim 1 wherein said  $C_{13}-C_{29}$  naphthene has a glass transition temperature in the range of  $-90^{\circ}$  to  $-30^{\circ}\text{C}$ . and contains, as a structural nucleus, a cyclohexyl hydrindan, di(cyclohexyl) alkane, adamantane, spirodecane, spiropentane, perhydrofluorene, perhydrobiphenyl, perhydroterphenyl, decalin, norbornane, perhydroindacene, perhydrohomotetraphthene, perhydroacenaphthene, perhydrophenanthrene, perhydrocrysene, perhydroindane-1-spirocyclohexane, perhydrocarylophylle, pinane, camphane, perhydrophenylnaphthalene or perhydro-  
pyrene.

6. The composition of claim 1 wherein said lubricant also contains an extreme pressure additive.

7. The composition of claim 6 wherein said extreme pressure additive consists essentially of a compound of phosphorus.

8. The composition of claim 7 wherein said extreme pressure additive consists essentially of tricresyl phosphate or a zinc dialkyl dithiophosphate, or mixtures thereof.

9. The composition of claim 1 wherein said naphthene comprises hydrogenated dimers and trimers of alpha-methyl styrene.

10. The composition of claim 1 wherein said  $C_3-C_8$  olefin in component (b) is at least one  $C_4$  olefin.

11. The composition of claim 10 wherein said  $C_4$  olefin consists essentially of isobutylene.

12. The composition of claim 9 wherein said blend contains from 0.1-20 parts by weight, based on said naphthene, of a hydrogenated polymer of a  $C_4$  mono-olefin.

13. The composition of claim 1 wherein said kinematic viscosity at  $210^{\circ}\text{F}$ ., is in the range of 5-50 c.s. and wherein the channel point is at least  $10^{\circ}\text{F}$ .

14. The composition of claim 3 also containing from 0.1-10 wt % of a synthetic sulfurized oil consisting essentially of a co-sulfurized blend of 90-30 parts of lard oil and 10-70 parts of an aliphatic olefin containing 12 to 128 carbon atoms.

5

10

15

30

35

40

45

50

55

60

65

15. The composition of claim 3 wherein said true oligomer of isobutylene has  $4N$  carbon atoms where  $N$  is an integer from 3-32 and has the formula



where  $n$  is an integer from 0 to 29 inclusive, and wherein  $z$  is:



or



or



or



or



16. The composition of claim 15 wherein said hydrocarbon base stock consists essentially of said oligomer of isobutylene.

17. The composition of claim 1 wherein said ester is a part ester which can produce an acidic pH in water.

18. The composition of claim 1 wherein said ester is of a linear aliphatic ethoxylated alcohol.

19. The composition of claim 1 wherein said ester consists essentially of mixed alkyl acid orthophosphate.

20. The composition of claim 19 and containing dilauryl phosphate.

\* \* \* \* \*